# EUROPEAN PATENT SPECIFICATION

(11) **EP 3 369 838 B1**
(45) Date of publication and mention of the grant of the patent: **21.08.2019**
(21) Application number: 16860213.4
(22) Date of filing: 26.10.2016
(51) Int. Cl.: C23C 2/06, C23C 2/14, C23C 2/16, C23C 2/18, C23C 2/20, C23C 2/26, C23C 2/40, C22C 18/04

(54) **ZINC ALLOY PLATED STEEL SHEET HAVING EXCELLENT BENDING WORKABILITY AND MANUFACTURING METHOD THEREFOR**
ZINKLEGIERTES STAHLBLECH MIT AUSGEZEICHNETER BIEGEBEARBEITBARKEIT UND HERSTELLUNGSVERFAHREN DAFÜR
TÔLE D'ACIER PLAQUÉE D'ALLIAGE DE ZINC PRÉSENTANT UNE EXCELLENTE APTITUDE AU CINTRAGE, ET SON PROCÉDÉ DE FABRICATION

(30) Priority: 26.10.2015 KR 20150148793
(43) Date of publication of application: 05.09.2018
(73) Proprietor: Posco, Pohang-si, Gyeongsangbuk-do 37859 (KR)
(72) Inventor: OH, Min-Suk, Gwangyang-si Jeollanam-do 57807 (KR); KIM, Sang-Heon, Gwangyang-si Jeollanam-do 57807 (KR); KIM, Tae-Chul, Gwangyang-si Jeollanam-do 57807 (KR); KIM, Jong-Sang, Gwangyang-si Jeollanam-do 57807 (KR); YUN, Hyun-Chu, Seoul 06194 (KR); YOO, Bong-Hwan, Gwangyang-si Jeollanam-do 57807 (KR)
(74) Representative: Zech, Stefan Markus
(86) International application number: PCT/KR2016/012098
(87) International publication number: WO 2017/074030

(56) References cited:
- EP-A1- 2 876 182
- WO-A2-2012/091385
- JP-B2- 3 212 977
- KR-A- 20120 075 235
- KR-A- 20150 052 376
- KR-A- 20150 052 376
- KR-B1- 101 500 043
- PISTOFIDIS, N. ET AL.: 'A Combined Microscopical and XRD Study of Zinc Coatings' SOLID STATE PHENOMENA vol. 163, 2010, pages 93 - 97, XP055482783

## Description

### [Technical Field]

The present disclosure relates to a zinc alloy plated steel sheet having high bending workability and a method for manufacturing the zinc alloy plated steel sheet.

### [Background Art]

A zinc plating method for suppressing the corrosion of iron by cathodic protection has high anti-corrosion efficiency and economic feasibility, and thus has been widely used in manufacturing steel materials having high corrosion resistance. Particularly, hot-dip zinc plated steel sheets, manufactured by dipping a steel material into molten zinc to form a plating layer, are obtainable through simple manufacturing processes and are relatively inexpensive, as compared to electro-zinc plated steel sheets, and thus, demand therefor has increased in a wide range of industries, such as the automotive industry, the home appliance industry, and the construction industry.

When a hot-dip zinc plated steel sheet is exposed to a corrosive environment, zinc having a lower oxidation-reduction potential than iron undergoes corrosion first, and thus, corrosion of the steel sheet is suppressed by sacrificial corrosion protection. Along with this, compact corrosion products are formed on the surface of the steel sheet as zinc of a plating layer is oxidized, thereby protecting the steel sheet from the corrosive environment and improving the corrosion resistance of the steel sheet.

However, air pollution and corrosive environments have increased with industrial advances, and regulations on resource and energy savings have been tightened. Therefore, the need to develop a steel material having higher corrosion resistance than existing zinc plated steel sheets has increased.

In this regard, research has been variously conducted into techniques for manufacturing zinc alloy-based plated steel sheets having corrosion resistance improved by adding elements such as aluminum (Al) and magnesium (Mg) to a zinc plating bath. Techniques for manufacturing a Zn-Al-Mg-based zinc alloy plated steel sheet, which is representative of zinc alloy-based plated steel sheets and manufactured by additionally adding magnesium (Mg) to a Zn-Al plating composition, have been actively researched.

However, such a Zn-Al-Mg-based zinc alloy plated steel sheet has poor bending workability. That is, the zinc alloy plated steel sheet includes large amounts of Zn-Al-Mg-based intermetallic compounds in a plating layer thereof as a result of thermodynamic reaction between zinc (Zn), aluminum (Al), and magnesium (Mg), and such intermetallic compounds may cause cracks in the plating layer during a bending process because of high hardness of the intermetallic compounds, thereby lowering the bending workability of the zinc alloy plated steel sheet.

Zinc alloy plated steel sheets and methods of manufacturing thereof are disclosed in WO 2012/091385 and EP 2 876 182.

### [Disclosure]

### [Technical Problem]

Aspects of the present disclosure provide, according to claim 1, a zinc alloy plated steel sheet having high bending workability and according to claim 10, a method for manufacturing the zinc alloy plated steel sheet. The scope of the present invention is defined by the appended claims.

### [Technical Solution]

According to an aspect of the present disclosure, a zinc alloy plated steel sheet may include a base steel sheet and a zinc alloy plating layer, wherein the zinc alloy plating layer may include a Zn single phase structure as a microstructure and a Zn-Al-Mg-based intermetallic compound, and the Zn single phase structure may have a degree (f) of (0001) preferred orientation, expressed by Formula 1 below, within a range of 50% or greater, $f \left(%\right) = \left({I}_{basal}/{I}_{total}\right) \times 100$ where Iₜₒₜₐₗ refers to an integral of all diffraction peaks of the Zn single phase structure when an X-ray diffraction pattern is measured within a range of 2 theta from 10° to 100° using a Cu-Kα source, and I_{basal} refers to an integral of diffraction peaks of the Zn single phase structure relating to a basal plane.

According to another aspect of the present disclosure, a method for manufacturing a zinc alloy plated steel sheet may include: preparing a zinc alloy plating bath including magnesium (Mg) and aluminum (Al); obtaining a zinc alloy plated steel sheet by dipping a base steel sheet into the zinc alloy plating bath to plate the base steel sheet; wiping the zinc alloy plated steel sheet with gas to adjust a plating weight; and after adjusting the plating weight of the zinc alloy plated steel sheet, cooling the zinc alloy plated steel sheet by spraying droplets of water or an aqueous solution onto the zinc alloy plated steel sheet and then using air, wherein when the droplets are sprayed, a droplet spray start temperature ranges from 405°C to 425°C, a droplet spray stop temperature ranges from 380°C to 400°C.

### [Advantageous Effects]

According to one of various effects of the present disclosure, an embodiment of the present disclosure provides a zinc alloy plated steel sheet having high bending workability as well as high corrosion resistance.

In addition, according to one of various effects of the present disclosure, the zinc alloy plated steel sheet of the embodiment has high surface quality.

In addition, according to one of various effects of the present disclosure, the zinc alloy plated steel sheet of the embodiment has high scratch resistance.

### [Description of Drawings]

FIGS. 1A and 1B are views illustrating results of an observation of a surface microstructure of Inventive Sample 1 and an observation of a surface microstructure of Comparative Sample 5.
FIGS. 2A and 2B are views illustrating results of an observation of a cross-sectional microstructure of Inventive Sample 1 and an observation of a cross-sectional microstructure of Comparative Sample 5.
FIG. 3 is a view illustrating results of X-ray diffractometer (XRD) analysis of Inventive Sample 1.

### [Best Mode]

Hereinafter, a zinc alloy plated steel sheet having high bending workability will be described in detail according to an aspect of the present disclosure.

According to the aspect of the present disclosure, the zinc alloy plated steel sheet includes a base steel sheet and a zinc alloy plating layer. In the present disclosure, the base steel sheet is not limited to a particular type. For example, a hot-rolled steel sheet or a cold-rolled steel sheet commonly used as a base steel sheet of a zinc alloy plated steel sheet may be used. However, hot-rolled steel sheets have a large amount of surface oxide scale that lowers plating adhesion and thus plating quality, and thus a hot-rolled steel sheet from which oxide scale has been previously removed using an acid solution may be used as the base steel sheet. In addition, the zinc alloy plating layer may be formed on one or each side of the base steel sheet.

The zinc alloy plating layer includes, by wt%, aluminum (Al): 0.5% to 3%, magnesium (Mg): 0.5% to 3%, and the balance of zinc (Zn) and inevitable impurities.

In the zinc alloy plating layer, magnesium (Mg) reacts with zinc (Zn) and aluminum (Al) and forms a Zn-Al-Mg-based intermetallic compound, thereby functioning as a key element improving the corrosion resistance of the zinc alloy plated steel sheet. If the content of magnesium (Mg) is excessively low, the Zn-Al-Mg-based intermetallic compound is not present in sufficient amounts in the microstructure of the zinc alloy plating layer, and thus corrosion resistance may not be sufficiently improved. Therefore, the amount of magnesium (Mg) in the zinc alloy plating layer is 0.5 wt% or greater, preferably 1.0 wt% or greater. However, if the content of magnesium (Mg) is excessively high, the effect of improving corrosion resistance is saturated, and Mg oxide dross having a negative effect on platability may be formed in a plating bath. In addition, the Zn-Al-Mg-based intermetallic compound having high harness may be formed in excessively large amounts in the microstructure of the zinc alloy plating layer, and thus bending workability may be lowered. Therefore, the amount of magnesium (Mg) in the zinc alloy plating layer is 3 wt% or less, preferably 2.9 wt% or less.

Aluminum (Al) suppresses the formation of Mg oxide dross and reacts with zinc (Zn) and magnesium (Mg) to form the Zn-Al-Mg-based intermetallic compound in the zinc alloy plating layer, thereby functioning as a key element improving the corrosion resistance of the zinc alloy plated steel sheet. If the content of aluminum (Al) is excessively low, the formation of Mg dross is not sufficiently suppressed, and the Zn-Al-Mg-based intermetallic compound is not present in sufficient amounts in the microstructure of the zinc alloy plating layer, which may result in insufficient improvements in corrosion resistance. Therefore, the amount of aluminum (Al) in the zinc alloy plating layer is 0.5 wt% or greater, preferably 0.6 wt% or greater. However, if the content of aluminum (Al) is excessively high, the effect of improving corrosion resistance is saturated, and the durability of plating equipment may be negatively affected because of a high plating bath temperature. Moreover, the Zn-Al-Mg-based intermetallic compound having high harness may be formed in excessively large amounts in the microstructure of the zinc alloy plating layer, and thus bending workability may be lowered. Therefore, the amount of aluminum (Al) in the zinc alloy plating layer is 3 wt% or less, preferably 2.6 wt% or less.

According to an embodiment, the contents of magnesium (Mg) and aluminum (Al) in the zinc alloy plating layer may satisfy the following Formula 2. If [Mg]/[Al] is 1.0 or less, scratch resistance may deteriorate, and if [Mg]/[Al] is greater than 4.0, Mg-based dross may be formed in large amounts in a hot-dip plating bath to lower workability. $1.0 < \left[Mg\right] / \left[Al\right] \leq 4.0$ where [Mg] and [Al] refer to the weight percentages (wt%) of corresponding elements, respectively.

The zinc alloy plating layer may include a Zn single phase structure as a microstructure and the Zn-Al-Mg-based intermetallic compound. In the present disclosure, the Zn-Al-Mg-based intermetallic compound is not limited to a particular type. However, for example, the Zn-Al-Mg-based intermetallic compound may include at least one selected from the group consisting of a Zn/Al/MgZn₂ ternary eutectic structure, a Zn/MgZn₂ binary eutectic structure, a Zn/Al binary eutectic structure, and an MgZn₂ single phase structure.

The inventors have conducted in-depth research into improving the bending workability of zinc alloy plated steel sheets and found that if a Zn single phase structure having a hexagonal close packing (HCP) structure is grown in a (0001) orientation in the microstructure of the zinc alloy plating layer, ductility increases owing to easy slippage, and thus cracks are markedly reduced in a bending process.

In the present disclosure, to obtain this effect, the degree (f) of (0001) preferred orientation, expressed by the following formula 1, is adjusted to be 50% or greater, more preferably 60% or greater. $f \left(%\right) = \left({I}_{basal}/{I}_{total}\right) \times 100$ where Iₜₒₜₐₗ refers to the integral of all diffraction peaks of the Zn single phase structure when an X-ray diffraction pattern is measured within the range of 2 theta from 10° to 100° using a Cu-Kα source, and I_{basal} refers to the integral of diffraction peaks of the Zn single phase structure relating to a basal plane.

In addition, the inventors have found that if the Zn single phase structure coarsely formed in the zinc alloy plating layer is refined in size, it is also helpful to reduce cracking during a bending process.

To obtain this effect of the present disclosure, the average grain diameter of the Zn single phase structure may be preferably adjusted to be 15 µm or less, more preferably 12 µm or less, and even more preferably 10 µm or less. The "average grain diameter" of the Zn single phase structure refers to the average of equivalent circular diameters of the Zn single phase structure measured by observing a thicknesswise cross-section of the zinc alloy plating layer.

The zinc alloy plated steel sheet of the present disclosure has high corrosion resistance and bending workability as well.

According to an embodiment, the zinc alloy plated steel sheet of the present disclosure may have a good appearance. Specifically, the number of black spots per unit area may be equal to or less than 0.1/cm² on the surface of the zinc alloy plated steel sheet.

To obtain these effects of the present disclosure, the area fraction of the Zn single phase structure may preferably be 40% or less (excluding 0%) on the surface of the zinc alloy plating layer. That is, the appearance of the zinc alloy plated steel sheet may be improved by maximizing the fraction of the Zn-Al-Mg-based intermetallic compound present on the surface of the zinc alloy plating layer.

According to an embodiment, the zinc alloy plated steel sheet of the present disclosure may also have high scratch resistance.

According to results of research conducted by the inventors, if the area fractions of the Zn/MgZn₂ binary eutectic structure and the Zn/Al/MgZn₂ ternary eutectic structure which have a layer structure and are present on the surface of the zinc alloy plating layer are maximized, scratch resistance may be markedly improved.

To obtain this effect of the present disclosure, preferably, the sum of the area fractions of the Zn/MgZn₂ binary eutectic structure and the Zn/Al/MgZn₂ ternary eutectic structure may be 50% or greater (excluding 100%), and the area fraction of the MgZn₂ single phase structure may be 10% or less (including 0%). The MgZn₂ single phase structure has high hardness and thus causes cracks during a machining process, and thus the area fraction of the MgZn₂ single phase structure may be adjusted to be as low as possible.

The zinc alloy plated steel sheet of the present disclosure may be manufactured by various methods without limitation. However, for example, when the zinc alloy plating layer solidifies from a molten state, the zinc alloy plating layer is cooled by spraying droplets thereon and then cooled with air to obtain the above-described degree of preferred orientation and average grain diameter.

In this case, droplets may be sprayed by a charge spray method to attach the droplets by electrostatic attraction between the droplets and the zinc alloy plated steel sheet. This charge spray method may be helpful in forming fine, uniform droplets and reducing the amount of droplets colliding with and bouncing off the zinc alloy plated steel sheet after being sprayed on the zinc alloy plated steel sheet, thereby facilitating rapid cooling of the zinc alloy plating layer from the molten state and having a positive effect on the growth of the Zn single phase structure in the (0001) orientation and refinement of the Zn single phase structure.

The droplets may be droplets of a phosphate aqueous solution capable of rapidly cooling the zinc alloy plating layer from the molten state through an endothermic reaction and thus effective in growing the Zn single phase structure in the (0001) orientation and refining the Zn single phase structure. Examples of the phosphate aqueous solution may include an aqueous solution of ammonium hydrogen phosphate ((NH₄)₂HPO₄), an aqueous solution of sodium ammonium hydrogen phosphate (NaNH₄HPO₄), an aqueous solution of zinc dihydrogen phosphate (Zn(H₂PO₄)₂), and an aqueous solution of calcium phosphate (Ca₃(PO₄)₂).

In addition, the content of the phosphate aqueous solution may be 1 wt% to 3 wt%. If the content of the phosphate aqueous solution is less than 1 wt%, the effect of the phosphate aqueous solution may not be sufficient. If the content of the phosphate aqueous solution is greater than 3 wt%, the effect of the phosphate aqueous solution is saturated, and nozzle clogging may occur in a continuous production process, lowering productivity.

In addition, the droplets are sprayed at a droplet spray start temperature of 405°C to 425°C, and more preferably 410°C to 420°C. Here, the term "droplet spray start temperature" refers to a surface temperature of the zinc alloy plated steel sheet at the start time of droplet spraying. If the droplet spray start temperature is less than 405°C, solidification of the Zn single phase structure may have already started, and thus black spots may be formed on the surface of the zinc alloy plated steel sheet. Conversely, if the droplet spray start temperature is greater than 425°C, droplets may not effectively undergo an endothermic reaction, and thus it may be difficult to obtain an intended structure.

In addition, the droplets are sprayed at a droplet spray stop temperature of 380°C to 400°C, and more preferably 390°C to 400°C. Here, the term "droplet spray stop temperature" refers to a surface temperature of the zinc alloy plated steel sheet at a point in time at which spraying of droplets stops. If the droplet spray stop temperature is greater than 400°C, an endothermic reaction by the droplets may occur ineffectively, and thus it may be difficult to obtain an intended structure. Conversely, if the droplet spray stop temperature is less than 380°C, a Mg₂Zn₁₁ phase may be formed due to over cooling while the Zn/MgZn₂ binary eutectic phase and the Zn/Al/MgZn₂ ternary phase start to solidify, and thus many black spots may be formed, decreasing the degree of (0001) preferred orientation of the Zn single phase structure.

In addition, the difference between the droplet spray start temperature and the droplet spray stop temperature may be 15°C or greater. If the difference is less than 15°C, the droplets may not undergo an effective endothermic reaction, and thus it may be difficult to obtain an intended structure.

In addition, the droplets may be sprayed in an amount of 50 g/m² to 100 g/m². If the spraying amount of the droplets is less than 50 g/m², the effect of the droplets may be insufficient, and if the spraying amount of the droplets is greater than 100 g/m², the effect of the droplets may be saturated.

### [Mode for Invention]

Hereinafter, the present disclosure will be described more specifically through examples.

### (Example 1)

Low carbon cold-rolled steel sheets each having a thickness of 0.8 mm, a width of 100 mm, and a length of 200 mm were prepared as base steel sheets for plating test samples, and then foreign substances such as rolling oil were removed from the surfaces of the base steel sheets by dipping the base steel sheets into acetone and washing the base steel sheets with ultrasonic waves. Thereafter, a 750°C reducing atmosphere heat treatment commonly performed to guarantee mechanical characteristics of steel sheets in the hot-dipping plating field was performed on the base steel sheets, and then the base steel sheets were dipped into plating baths (bath temperature: 460°C) having compositions shown in Table 1 below to fabricate zinc alloy plated steel sheets. Thereafter, each of the zinc alloy plated steel sheets was wiped with gas to adjust a plating weight to be 70 g/m² on each side. Then, the zinc alloy plated steel sheets were cooled under the conditions shown in Table 1 below and were cooled with air. Although not shown in Table 1 below, Comparative Sample 5 was prepared by performing a gas wiping process on a zinc alloy plated steel sheet fabricated using the same plating bath as that used to fabricate Inventive Sample 1 to adjust a plating weight to be 70 g/m² on each side, and then cooling the zinc alloy plated steel sheet using a general cooling device at an average cooling rate of 12°C/sec until the plating layer of the zinc alloy plated steel sheet was completely solidified (at about 300°C or less).

Then, the microstructures of the fabricated zinc alloy plated steel sheets were observed using an FE-SEM (SUPRA-55VP, Zeiss) as illustrated in FIGS. 1 and 2, and the average grain diameter of a Zn single phase structure of each of the zinc alloy plated steel sheets was measured as shown in Table 2 below.

Thereafter, the degree (f) of (0001) preferred orientation of the Zn single phase structure was measured using the following Formula 1, and results thereof are shown in Table 2 below. $f \left(%\right) = \left({I}_{basal}/{I}_{total}\right) \times 100$ where Iₜₒₜₐₗ refers to the integral of all diffraction peaks of the Zn single phase structure when an X-ray diffraction pattern was measured within the range of 2 theta from 10° to 100° using a Cu-Kα source, and I_{basal} refers to the integral of diffraction peaks of the Zn single phase structure relating to a basal plane.

Thereafter, the bending workability of each of the zinc alloy plated steel sheets was evaluated, and results thereof are shown in Table 2 below.

Corrosion resistance was evaluated as follows.

A salt spray test (based on KS-C-0223) was performed on each of the zinc alloy plated steel sheets to facilitate corrosion, and then the time taken until the area fraction of red rust on the surface of each plating layer was 5% was measured.

Bending workability was evaluated as follows.

3T bending was performed on each of the zinc alloy plated steel sheets, and a 1-mm length of the apex of each bent portion was observed using an SEM to measure the area fraction of bending cracks using an image analysis system.

**[Table 1]**

| No. | Composition of plating bath (wt%) | | Droplet spray start temperature (°C) | Droplet spray stop temperature (°C) | Droplets | Spraying amount (g/m²) | Notes |
|---|---|---|---|---|---|---|---|
| | Al | Mg | | | | | |
| 1 | 1.6 | 1.6 | 410 | 390 | Aqueous solution of ammonium hydrogen phosphate, 2 wt% | 70 | *IS 1 |
| 2 | 1.6 | 1.6 | 420 | 400 | Aqueous solution of ammonium hydrogen phosphate, 2 wt% | 70 | IS 2 |
| 3 | 1.6 | 1.6 | **430** | 400 | Aqueous solution of ammonium hydrogen phosphate, 2 wt% | 70 | **CS 1 |
| 4 | 1.6 | 1.6 | **400** | 390 | Aqueous solution of ammonium hydrogen phosphate, 2 wt% | 70 | CS 2 |
| 5 | 1.6 | 1.6 | 420 | **405** | Aqueous solution of ammonium hydrogen phosphate, 2 wt% | 70 | CS 3 |
| 6 | 1.6 | 1.6 | 410 | **375** | Aqueous solution of ammonium hydrogen phosphate, 2 wt% | 70 | CS 4 |

| | | | | | | | |
|---|---|---|---|---|---|---|---|
| *IS: Inventive Sample, **CS: Comparative Sample | | | | | | | |

**[Table 2]**

| No. | Average grain diameter of Zn single phase structure (µm) | f(%) | Red rust occurrence time (h) | Area fraction of bending cracks (%) | Notes |
|---|---|---|---|---|---|
| 1 | 8 | 63 | 650 | 8 | *IS 1 |
| 2 | 10 | 62 | 645 | 9 | IS 2 |
| 3 | 12 | 49 | 640 | 25 | **CS 1 |
| 4 | 14 | 47 | 630 | 38 | CS 2 |
| 5 | 15 | 46 | 620 | 40 | CS 3 |
| 6 | 16 | 44 | 610 | 42 | CS 4 |
| 7 | 18 | 42 | 600 | 45 | CS 5 |

| | | | | | |
|---|---|---|---|---|---|
| *IS: Inventive Sample, **CS: Comparative Sample | | | | | |

Referring to Table 2, Inventive Samples 1 and 2 satisfying conditions proposed in the present disclosure had high bending workability.

However, although Comparative Samples 1 to 5 had high corrosion resistance, Comparative Samples 1 to 5 had poor bending workability because the (f) values thereof were less than 50%.

FIG. 1A and 1B are views illustrating results of an observation of a surface microstructure of Inventive Sample 1 of the present disclosure and an observation of a surface microstructure of Comparative Sample 5, and FIGS. 2A and 2B are views illustrating results of an observation of a cross-sectional microstructure of Inventive Sample 1 of the present disclosure and an observation of a cross-sectional microstructure of Comparative Sample 5.

FIG. 3 is a view illustrating results of X-ray diffractometer (XRD) analysis of Inventive Sample 1. In FIG. 3, peaks denoted with "○ and "●" are all diffraction peaks of the Zn single phase structure, and the peaks denoted with "○" are diffraction peaks of the Zn single phase structure relating to a basal plane.

### (Example 2)

Low carbon cold-rolled steel sheets each having a thickness of 0.8 mm, a width of 100 mm, and a length of 200 mm were prepared as base steel sheets for plating test samples, and then foreign substances such as rolling oil were removed from the surfaces of the base steel sheets by dipping the base steel sheets into acetone and washing the base steel sheets with ultrasonic waves. Thereafter, a 750°C reducing atmosphere heat treatment commonly performed to guarantee mechanical characteristics of steel sheets in the hot-dipping plating field was performed on the base steel sheets, and then the base steel sheets were dipped into plating baths having compositions shown in Table 3 below to fabricate zinc alloy plated steel sheets. Thereafter, each of the zinc alloy plated steel sheets was wiped with gas to adjust a plating weight to be 70 g/m² on each side. Then, the zinc alloy plated steel sheets were cooled under the same conditions as Inventive Sample 1 of Example 1.

Thereafter, the fractions of microstructures observed on the surface of each of the zinc alloy plated steel sheets were measured, and the number of black spots on the surface of each of the zinc alloy plated steel sheets was measured. Results thereof are shown in Tables 3 and 4.

Thereafter, a friction test (linear friction test) was performed by rubbing the surface of each of the zinc alloy plated steel sheets 20 times with a tool head at a constant pressure. In the friction test, a target load was 333.3 kgf, a pressure was 3.736 MPa, the tool head traveled 200 mm per rub, and the speed of the tool head was 20 mm/s.

After the friction test, a stripping test was performed on each of the zinc alloy plated steel sheets. Specifically, cellophane adhesive tape (NB-1 by Ichiban) was attached to a bent portion of each of the zinc alloy plated steel sheets subjected to a 10R bending process, and then the cellophane tape was momentarily separated. Then, the number of plating layer defects was measured using an optical microscope (magnification: 50 times). Results of the measurement were evaluated as "○" when the number of plating layer defects was 5/m² or less, and "X" when the number of plating layer defects was greater than 5/m². Evaluation results are shown in Table 4 below.

In addition, after the friction test, each of the zinc alloy plated steel sheets was inserted into a salt spray tester, and the time taken until the occurrence of red rust was measured according to international standard ASTM B117-11. In that time, a 5% salt solution (35°C, pH 6.8) was sprayed at a rate of 2 ml/80 cm² per hour. When the time taken until red rust was present on a sample was 500 hours or greater, the sample was evaluated as "○", and when the time taken until red rust was present on a sample was less than 500, the sample was evaluated as "X." Results of the evaluation are shown in Table 4 below.

**[Table 3]**

| No. | Alloy composition (wt%) | | | Area fractions of surface structures (area%) | | | | | | Notes |
|---|---|---|---|---|---|---|---|---|---|---|
| | Al | Mg | Mg/Al | Zn | Zn/MgZn₂ | Zn/Al/MgZn₂ | MgZn₂ | Zn/Al | Zn/Al/MgZn₂ + Zn/MgZn₂ | |
| 1 | 0.6 | 2.3 | 3.83 | 28 | 41 | 31 | 0 | 0 | 72 | *IS A |
| 2 | 1.5 | 2.8 | 1.87 | 20 | 57 | 21 | 1 | 1 | 78 | IS B |
| 3 | 2 | 2.9 | 1.45 | 8 | 63 | 28 | 1 | 0 | 91 | IS C |
| 4 | 2.2 | 2.7 | 1.23 | 4 | 58 | 34 | 2 | 2 | 92 | IS D |
| 5 | 2.6 | 2.9 | 1.12 | 4 | 39 | 51 | 3 | 3 | 90 | IS E |
| 6 | 0 | 0 | - | 100 | 0 | 0 | 0 | 0 | 0 | **CS A |
| 7 | 1.4 | 1 | 0.71 | 82 | 7 | 11 | 0 | 0 | 18 | CS B |
| 8 | 2.5 | 1.2 | 0.48 | 6 | 21 | 26 | 46 | 1 | 47 | CS C |
| 9 | 5 | 0 | 0.00 | 76 | 0 | 0 | 0 | 24 | 0 | CS D |
| 10 | 5 | 1 | 0.20 | 59 | 9 | 11 | 0 | 21 | 20 | CS E |
| 11 | 8 | 3 | 0.38 | 13 | 7 | 13 | 18 | 49 | 20 | CS F |
| 12 | 55 | 0 | 0.00 | 14 | 0 | 0 | 0 | 86 | 0 | CS G |
| Here, surface structures refer to microstructures observed on the surfaces of zinc alloy plating layers. | | | | | | | | | | |

| | | | | | | | | | | |
|---|---|---|---|---|---|---|---|---|---|---|
| *IS: Inventive Sample, **CS: Comparative Sample | | | | | | | | | | |

**[Table 4]**

| No. | Number of black spots (/cm²) | Results of stripping test after friction test | | Results of salt spray test after friction test | | Notes |
|---|---|---|---|---|---|---|
| | | Number of defects (/m²) | Evaluation results | Red rust occurrence time (hour) | Evaluation results | |
| 1 | 0.05 | 3 | ○ | 520 | ○ | *IS A |
| 2 | 0.08 | 2 | ○ | 550 | ○ | IS B |
| 3 | 0.04 | 4 | ○ | 600 | ○ | IS C |
| 4 | 0.08 | 3 | ○ | 650 | ○ | IS D |
| 5 | 0.04 | 2 | ○ | 580 | ○ | IS E |
| 6 | 1.2 | 2 | ○ | 120 | X | **CS A |
| 7 | 0.8 | 3 | ○ | 230 | X | CS B |
| 8 | 0.05 | 23 | X | 620 | ○ | CS C |
| 9 | 1.1 | 3 | ○ | 350 | X | CS D |
| 10 | 0.6 | 2 | ○ | 420 | X | CS E |
| 11 | 0.06 | 15 | X | 650 | ○ | CS F |
| 12 | 0.05 | 11 | X | 200 | X | CS G |

| | | | | | | |
|---|---|---|---|---|---|---|
| *IS: Inventive Sample, **CS: Comparative Sample | | | | | | |

Referring to Table 4, Inventive Samples A to E satisfying conditions proposed in the present disclosure had good appearance and high scratch resistance.

However, each of Comparative Samples A, B, D, and E had poor appearance because the area fraction of a Zn single phase structure present on the surface of a plating layer was excessively high, and each of Comparative Samples A to G had poor scratch resistance because the area fractions of a Zn/MgZn₂ binary eutectic structure and a Zn/Al/MgZn₂ ternary eutectic structure are excessively low.

## Claims

1. A zinc alloy plated steel sheet comprising a base steel sheet and a zinc alloy plating layer,
wherein the zinc alloy plating layer comprises by wt%, aluminum (Al): 0.5% to 3%, magnesium (Mg): 0.5% to 3%, and a balance of zinc (Zn) and inevitable impurities, and the zinc alloy plating layer comprises a Zn single phase structure as a microstructure and a Zn-Al-Mg-based intermetallic compound, and
the Zn single phase structure has a degree (f) of (0001) preferred orientation, expressed by Formula 1 below, within a range of 50% or greater, $f \left(%\right) = \left({I}_{basal}/{I}_{total}\right) \times 100$ where Iₜₒₜₐₗ refers to an integral of all diffraction peaks of the Zn single phase structure when an X-ray diffraction pattern is measured within a range of 2 theta from 10° to 100° using a Cu-Kα source, and I_{basal} refers to an integral of diffraction peaks of the Zn single phase structure relating to a basal plane.

2. The zinc alloy plated steel sheet of claim 1, wherein the Zn single phase structure has a degree (f) of (0001) preferred orientation, expressed by Formula 1, within a range of 60% or greater.

3. The zinc alloy plated steel sheet of claim 1, wherein the Zn-Al-Mg-based intermetallic compound comprises at least one selected from the group consisting of a Zn/MgZn₂ binary eutectic structure, a Zn/Al binary eutectic structure, an MgZn₂ single phase structure, and a Zn/Al/MgZn₂ ternary eutectic structure.

4. The zinc alloy plated steel sheet of claim 1, wherein an area fraction of the Zn single phase structure on a surface of the zinc alloy plating layer is 40% or less, excluding 0%.

5. The zinc alloy plated steel sheet of claim 1, wherein a total area fraction of a Zn/MgZn₂ binary eutectic structure and a Zn/Al/MgZn₂ ternary eutectic structure is 50% or greater, excluding 100%, on a surface of the zinc alloy plating layer.

6. The zinc alloy plated steel sheet of claim 1, wherein an area fraction of an MgZn₂ single phase structure on a surface of the zinc alloy plating layer is 10% or less, excluding 0%.

7. The zinc alloy plated steel sheet of claim 1, wherein an average grain diameter of the Zn single phase structure observed on a cross-section of the zinc alloy plating layer taken in a sheet thickness direction is 15 µm or less, excluding 0 µm.

8. The zinc alloy plated steel sheet of claim 1, wherein the zinc alloy plating layer satisfies Formula 2 below: $1.0 < \left[Mg\right] / \left[Al\right] \leq 4.0$ where [Mg] and [Al] refer to weight percentages (wt%) of corresponding elements, respectively.

9. The zinc alloy plated steel sheet of claim 1, wherein a number of black spots per unit area is 0.1/cm² or less on a surface of the zinc alloy plated steel sheet.

10. A method for manufacturing a zinc alloy plated steel sheet, the method comprising:
preparing a zinc alloy plating bath comprising by wt%, aluminum (Al): 0.5% to 3%, magnesium (Mg): 0.5% to 3%, and a balance of zinc (Zn) and inevitable impurities;
obtaining a zinc alloy plated steel sheet by dipping a base steel sheet into the zinc alloy plating bath to plate the base steel sheet;
wiping the zinc alloy plated steel sheet with gas to adjust a plating weight; and
after adjusting the plating weight of the zinc alloy plated steel sheet, cooling the zinc alloy plated steel sheet by spraying droplets of water or an aqueous solution onto the zinc alloy plated steel sheet and then using air,
wherein when the droplets are sprayed, a droplet spray start temperature ranges from 405°C to 425°C, a droplet spray stop temperature ranges from 380°C to 400°C.

11. The method of claim 10, wherein when the droplets are sprayed, a difference between the droplet spray start temperature and the droplet spray stop temperature is 15°C or greater.

12. The method of claim 10, wherein the droplets are sprayed by a charge spray method to attach the droplets by electrostatic attraction between the droplets and the zinc alloy plated steel sheet.

13. The method of claim 10, wherein the droplets are sprayed in an amount of 50 g/m² to 100 g/m².

14. The method of claim 10, wherein the aqueous solution is a phosphate aqueous solution.

15. The method of claim 14, wherein the phosphate aqueous solution comprises at least one selected from the group consisting of an aqueous solution of ammonium hydrogen phosphate ((NH₄)₂HPO₄), an aqueous solution of sodium ammonium hydrogen phosphate (NaNH₄HPO₄), an aqueous solution of zinc dihydrogen phosphate (Zn(H₂PO₄)₂), and an aqueous solution of calcium phosphate (Ca₃(PO₄)₂).

16. The method of claim 14, wherein the phosphate aqueous solution has a concentration of 1 wt% to 3 wt%.

## Patentansprüche

1. Mit Zinklegierung plattiertes Stahlblech, umfassend ein Basisstahlblech und eine Zinklegierungsplattierungsschicht,
wobei die Zinklegierungsplattierungsschicht in Gewichts-% Aluminium (A|): 0,5 % bis 3 %, Magnesium (Mg): 0,5 % bis 3 % und einen Rest aus Zink (Zn) und unvermeidbaren Verunreinigungen umfasst, und die Zinklegierungsplattierungsschicht eine Zn-Einzelphasenstruktur als Mikrostruktur und eine intermetallische Verbindung auf Zn-Al-Mg-Basis umfasst, und
die Zn-Einzelphasenstruktur einen Grad (f) an (0001) Vorzugsorientierung, die durch die nachstehende Formel 1 ausgedrückt ist, innerhalb eines Bereichs von 50 % oder mehr hat, $f \left(%\right) = \left({I}_{basal}/{I}_{total}\right) \times 100$ worin sich Iₜₒₜₐₗ auf ein Integral aller Beugungsspitzen der Zn-Einzelphasenstruktur bezieht, wenn ein Röntgenbeugungsmuster innerhalb eines Bereichs von 2 Theta von 10° bis 100° unter Verwendung einer Cu-Kα-Quelle gemessen wird, und sich I_{basal} auf ein Integral von Beugungsspitzen der Zn-Einzelphasenstruktur bezieht, das sich auf eine Basalebene bezieht.

2. Mit Zinklegierung plattiertes Stahlblech nach Anspruch 1, wobei die Zn-Einzelphasenstruktur einen Grad (f) an (0001) Vorzugsorientierung, die durch die Formel 1 ausgedrückt ist, innerhalb eines Bereichs von 60 % oder mehr hat.

3. Mit Zinklegierung plattiertes Stahlblech nach Anspruch 1, wobei die intermetallische Verbindung auf Zn-Al-Mg-Basis mindestens eine Struktur hat, die aus der Gruppe ausgewählt ist, die aus einer binären eutektischen Struktur aus Zn/MgZn₂, einer binären eutektischen Struktur aus Zn/Al, einer MgZn₂-Einzelphasenstruktur und einer ternären eutektischen Struktur aus Zn/Al/MgZn₂ besteht.

4. Mit Zinklegierung plattiertes Stahlblech nach Anspruch 1, wobei ein Flächenanteil der Zn-Einzelphasenstruktur auf einer Oberfläche der Zinklegierungsplattierungsschicht 40 % oder weniger, 0 % ausgeschlossen, beträgt.

5. Mit Zinklegierung plattiertes Stahlblech nach Anspruch 1, wobei ein Gesamtflächenanteil einer binären eutektischen Struktur aus Zn/MgZn₂ und einer ternären eutektische Struktur aus Zn/Al/MgZn₂ 50 % oder mehr, 100 % ausgeschlossen, auf einer Oberfläche der Zinklegierungsplattierungsschicht beträgt.

6. Mit Zinklegierung plattiertes Stahlblech nach Anspruch 1, wobei ein Flächenanteil einer MgZn₂-Einzelphasenstruktur auf einer Oberfläche der Zinklegierungsplattierungsschicht 10 % oder weniger, 0 % ausgeschlossen, beträgt.

7. Mit Zinklegierung plattiertes Stahlblech nach Anspruch 1, wobei ein mittlerer Korndurchmesser der Zn-Einzelphasenstruktur, der an einem in einer Blechdickenrichtung ermittelten Querschnitt der Zinklegierungsplattierungsschicht beobachtet wurde, 15 µm oder weniger, 0 µm ausgeschlossen, beträgt.

8. Mit Zinklegierung plattiertes Stahlblech nach Anspruch 1, wobei die Zinklegierungsplattierungsschicht die nachstehende Formel 2 erfüllt: $1,0 < \left[Mg\right] / \left[Al\right] \leq 4,0 ,$ worin sich [Mg] und [Al] jeweils auf die Gewichtsprozente (Gew.-%) der entsprechenden Elemente beziehen.

9. Mit Zinklegierung plattiertes Stahlblech nach Anspruch 1, wobei eine Anzahl schwarzer Flecken pro Einheitsfläche 0,1/cm² oder weniger auf einer Oberfläche des Zinklegierungsplattierungsschicht beträgt.

10. Verfahren zum Herstellen eines mit Zinklegierung plattierten Stahlblechs, wobei das Verfahren umfasst:
Vorbereiten eines Zinklegierungsplattierungsbads, das in Gew.-% Aluminium (Al): 0,5 % bis 3 %, Magnesium (Mg): 0,5 % bis 3 % und einen Rest aus Zink (Zn) und unvermeidbaren Verunreinigungen umfasst,
Erhalten eines mit Zinklegierung plattierten Stahlblechs durch Eintauchen eines Basisstahlblechs in das Zinklegierungsplattierungsbad, um das Basisstahlblech zu plattieren;
Abstreifen des mit Zinklegierung plattierten Stahlblechs mit Gas, um ein Plattierungsgewicht anzupassen; und
Nach dem Anpassen des Plattierungsgewichts des mit Zinklegierung plattierten Stahlblechs, Abkühlen des mit Zinklegierung plattierten Stahlblechs, indem Wassertröpfchen oder eine wässrige Lösung auf das mit Zinklegierung plattierten Stahlblech aufgesprüht werden und dann Luft verwendet wird,
wobei, wenn die Tröpfchen aufgesprüht werden, eine Tröpfchensprühbeginntemperatur von 405° C bis 425° C reicht, eine Tröpfchensprühstopptemperatur von 380° C bis 400° C reicht.

11. Verfahren nach Anspruch 10, wobei, wenn die Tröpfchen aufgesprüht werden, ein Unterschied zwischen der Tröpfchensprühbeginntemperatur und der Tröpfchensprühstopptemperatur 15° C oder mehr beträgt.

12. Verfahren nach Anspruch 10, wobei die Tröpfchen durch ein Ladungssprühverfahren aufgesprüht werden, um die Tröpfchen durch elektrostatische Anziehung zwischen den Tröpfchen und dem mit Zinklegierung plattierten Stahlblech anhaften zu lassen.

13. Verfahren nach Anspruch 10, wobei die Tröpfchen in einer Menge von 50 g/m² bis 100 g/m² aufgesprüht werden.

14. Verfahren nach Anspruch 10, wobei es sich bei der wässrigen Lösung um eine wässrige Phosphatlösung handelt.

15. Verfahren nach Anspruch 14, wobei die wässrige Phosphatlösung mindestens eine wässrige Lösung umfasst, die aus der Gruppe ausgewählt ist, die aus einer wässrigen Lösung aus Ammoniumhydrogenphosphat ((NH₄)₂HPO₄), einer wässrigen Lösung aus Natriumammoniumhydrogenphosphat (NaNH₄HPO₄), einer wässrigen Lösung aus Zinkdihydrogenphosphat (Zn(H₂PO₄)₂) und einer wässrigen Lösung aus Calciumphosphat (Ca₃(PO₄)₂) besteht.

16. Verfahren nach Anspruch 14, wobei die wässrige Phosphatlösung eine Konzentration von 1 Gew.-% bis 3 Gew.-% hat.

## Revendications

1. Tôle d'acier plaquée en alliage de zinc comprenant une tôle d'acier de base et une couche de placage en alliage de zinc,
sachant que la couche de placage en alliage de zinc comprend, en % de poids, de l'aluminium (Al) : 0,5 % à 3 %, du magnésium (Mg) : 0,5 % à 3 %, et un solde de zinc (Zn) et d'impuretés inévitables, et la couche de placage en alliage de zinc comprend une structure monophasée de Zn comme microstructure et un composé intermétallique à base de Zn-Al-Mg, et
la structure monophasée de Zn a un degré (f) d'orientation préférée (0001), exprimé par la Formule 1 ci-dessous, compris dans une plage de 50 % ou plus, $f \left(%\right) = \left({I}_{basal}/{I}_{total}\right) \times 100$ où Iₜₒₜₐₗ se rapporte à une intégrale de tous les pics de diffraction de la structure monophasée de Zn lorsqu'un motif de diffraction par rayons X est mesuré dans une plage de 2 théta de 10° à 100° moyennant une source de Cu-Kα, et I_{basal} se rapporte à une intégrale de pics de diffraction de la structure monophasée de Zn relatifs à un plan basal.

2. La tôle d'acier plaquée en alliage de zinc de la revendication 1, sachant que la structure monophasée de Zn a un degré (f) d'orientation préférée (0001), exprimé par la Formule 1, compris dans une plage de 60 % ou plus.

3. La tôle d'acier plaquée en alliage de zinc de la revendication 1, sachant que le composé intermétallique à base de Zn-Al-Mg comprend au moins une structure sélectionnée dans le groupe constitué par une structure eutectique binaire de Zn/MgZn₂, une structure monophasée de MgZn₂, et une structure eutectique ternaire de Zn/Al/MgZn₂.

4. La tôle d'acier plaquée en alliage de zinc de la revendication 1, sachant qu'une fraction d'aire de la structure monophasée de Zn sur une surface de la couche de placage en alliage de zinc est de 40 % ou moins, à l'exception de 0 %.

5. La tôle d'acier plaquée en alliage de zinc de la revendication 1, sachant qu'une fraction d'aire totale d'une structure eutectique binaire de Zn/MgZn₂ et d'une structure eutectique ternaire de Zn/Al/MgZn₂ est de 50 % ou plus, à l'exception de 100 %, sur une surface de la couche de placage en alliage de zinc.

6. La tôle d'acier plaquée en alliage de zinc de la revendication 1, sachant qu'une fraction d'aire d'une structure monophasée de MgZn₂ sur une surface de la couche de placage en alliage de zinc est de 10 % ou moins, à l'exception de 0 %.

7. La tôle d'acier plaquée en alliage de zinc de la revendication 1, sachant qu'un diamètre de grain moyen de la structure monophasée de Zn observé sur une section transversale de la couche de placage en alliage de zinc pris dans une direction d'épaisseur de tôle est de 15 µm ou moins, à l'exception de 0 µm.

8. La tôle d'acier plaquée en alliage de zinc de la revendication 1, sachant que la couche de placage en alliage de zinc satisfait à la Formule 2 ci-dessous : $1,0 < \left[Mg\right] / \left[Al\right] \leq 4,0$ où [Mg] et [Al] se rapportent à des pourcentages de poids (% de poids) d'éléments correspondants, respectivement.

9. La tôle d'acier plaquée en alliage de zinc de la revendication 1, sachant qu'un nombre de tâches noires par unité d'aire est de 0,1/cm² ou moins sur une surface de la tôle d'acier plaquée en alliage de zinc.

10. Procédé de fabrication d'une tôle d'acier plaquée en alliage de zinc, le procédé comprenant :
la préparation d'un bain de placage en alliage de zinc comprenant, en % de poids, de l'aluminium (Al) : 0,5 % à 3 %, du magnésium (Mg) : 0,5 % à 3 %, et un solde de zinc (Zn) et d'impuretés inévitables ;
l'obtention d'une tôle d'acier plaquée en alliage de zinc par immersion d'une tôle d'acier de base dans le bain de placage en alliage de zinc pour plaquer la tôle d'acier de base ;
le balayage de la tôle d'acier plaquée en alliage de zinc avec du gaz pour ajuster un poids de placage ; et
après l'ajustage du poids de placage de la tôle d'acier plaquée en alliage de zinc, le refroidissement de la tôle d'acier plaquée en alliage de zinc par pulvérisation de gouttelettes d'eau ou d'une solution aqueuse sur la tôle d'acier plaquée en alliage de zinc et ensuite avec de l'air,
sachant que lorsque les gouttelettes sont pulvérisées, une température de départ de pulvérisation de gouttelettes va de 405 °C à 425 °C, une température d'arrêt de pulvérisation de gouttelettes va de 380 °C à 400 °C.

11. Le procédé de la revendication 10, sachant que lorsque les gouttelettes sont pulvérisées, une différence entre la température de départ de pulvérisation de gouttelettes et la température d'arrêt de pulvérisation de gouttelettes est de 15 °C ou supérieure.

12. Le procédé de la revendication 10, sachant que les gouttelettes sont pulvérisées par un procédé de pulvérisation de charge pour fixer les gouttelettes par attraction électrostatique entre les gouttelettes et la tôle d'acier plaquée en alliage de zinc.

13. Le procédé de la revendication 10, sachant que les gouttelettes sont pulvérisées dans une quantité de 50 g/m² à 100 g/m².

14. Le procédé de la revendication 10, sachant que la solution aqueuse est une solution aqueuse de phosphate.

15. Le procédé de la revendication 14, sachant que la solution aqueuse de phosphate comprend au moins une solution sélectionnée dans le groupe constitué par une solution aqueuse de phosphate d'hydrogène d'ammonium ((NH₄)₂HPO₄), une solution aqueuse de phosphate d'hydrogène d'ammonium de sodium (NaNH₄HPO₄), une solution aqueuse de phosphate de dihydrogène de zinc (Zn(H₂PO₄)₂), et une solution aqueuse de phosphate de calcium (Ca₃(PO₄)₂).

16. Le procédé de la revendication 14, sachant que la solution aqueuse de phosphate a une concentration de 1 % de poids à 3 % de poids.
